

## UNITED STATES PATENT OFFICE

2,346,357

## HIGH TEMPERATURE LUBRICANT

Robert E. Burk and Everett C. Hughes, Cleveland Heights, Ohio, assignors to The Standard Oil Company, Cleveland, Ohio, a corporation of Ohio

No Drawing. Application December 24, 1941,  
Serial No. 424,362

4 Claims. (Cl. 252—35)

This invention relates to lubricants; and it is among the objects of the invention to provide improved lubrication in high temperature, such as in internal combustion engines. Other objects and advantages will appear as the description proceeds.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The lubricant base may be a usual lubricating oil of viscosity desired in view of particular duty contemplated, or for instance 45 to 200 sec. S. U. at 210° F. We have found that salts of metals having oxidation activity or which are oxidation catalysts not particularly at crank-case temperature but at higher temperature, promote diminution of carbonaceous deposits outstandingly, and in combination with what we term an "anti-oxidant" give results much better than the total of the respective agents alone, "anti-oxidant" here having a meaning not as with gasoline but as an inhibitor for metal catalysts such as iron, copper, or lead. It is particularly remarkable that an agent of oxidizing character and whose activity tends primarily to be antagonistic to anti-oxidant action should work to these ends. The salts of metals constituting the oxidation catalysts comprise: naphthenates; salts of acid radicals such as of tall oil or sulphurized tall oil; acids derived from the oxidation of petroleum fractions or polymers; xanthic, i. e., acids of the type

—S  
ROC—SH

in which R is alkyl, aryl, alkaryl and sufficient to solubilize the metal compound; medium molecular weight fatty acids chosen so that the resulting salt will have 15—30 carbon atoms; acids derived from saponified wool fat (degras) with or without the alcohol, and the wool fat may be sulphurized, e. g., with  $P_2S_5$ , before or after hydrolysis, and for conciseness such acids are hereinafter designated "organic acids of low volatility" the stated salts of which promote diminution of carbonaceous deposits. The naphthenates may also be chlorinated or halogenated, and in some cases sulphurized. The metals above referred to are chromium, also vanadium, manganese, cobalt and molybdenum. In general,  $\frac{1}{2}$  to 2 per cent, or more, up to 3 per cent of the metal compound

may be used. There is a distinction in favor of the chromium compounds over the others, and particularly cobalt. A chromium salt or naphthenate is especially characterized by catalyzing the combustion and elimination of carbonaceous deposits at combustion zone temperatures, while inhibiting deterioration of oil at crank-case temperatures in the presence of iron and copper. The other naphthenates or salts have a tendency to also promote the oxidation or deterioration of oil at crank-case temperatures in the presence of iron and copper, and cannot be advantageously used alone in oil as in the case of the chromium compounds, but they require further corrective additions. The chromium compounds also may be used with the said anti-oxidant agents. These agents comprise: nitrogen-containing diphenyl methane derivatives, i. e., tetramethyl diamino diphenyl methane, diamino diphenyl methane, and analogues, also sulphur-containing compounds such as  $P_2S_5$  treated degras,  $P_2S_5$  treated polyolefins,  $P_2S_5$  treated distilled cashew nut shell oil, etc. Up to 3 per cent, preferably  $\frac{1}{4}$  to 2 per cent of such agent additive to the metal compounds may be employed. Particularly the vanadium, manganese and cobalt salts are aided by the presence of the diamino diphenyl methane derivatives. A peculiarity is that such derivatives used with the vanadium, manganese or cobalt salts are found to reduce crank-case temperature oxidation without being detrimental to the activity of the carbon combustion properties at combustion zone temperature, but a further peculiarity is that the latter property is destroyed by the sulphur-containing additives except with the chromium salt. Further, the corrosive tendencies of the metal naphthenates, particularly of cobalt, vanadium and manganese, toward bearing metals and copper is reduced by tetramethyl diamino diphenyl methane, and peculiarly it is found to be completely eliminated by the further inclusion of less than  $\frac{1}{4}$  per cent of diamino diphenyl methane.

As an example: A lubricant is made up of S. A. E. 20 lubricating oil and 0.5 per cent of chromium naphthenate and 1.5 per cent of the reaction product of  $P_2S_5$  on degras.

As another example: A lubricant is made up of a similar oil and 0.5 per cent of cobalt naphthenate and 1.5 per cent of tetramethyl diamino diphenyl methane.

As another example: A lubricant is made up with a similar oil and 0.5 per cent of chromium naphthenate and 2 per cent of the reaction product of  $P_2S_5$  on polyolefin.

As another example: With a similar lubricating oil there is incorporated chromium naphthalene  $\frac{1}{2}$  per cent and tetramethyl diamino diphenyl methane  $\frac{1}{2}$ -2 per cent.

As another example: With a similar lubricating oil there is incorporated vanadyl naphthalene  $\frac{1}{2}$  per cent and tetramethyl diamino diphenyl methane  $\frac{1}{2}$ -2 per cent, and diamino diphenyl methane 0.15 per cent.

As another example: With a similar lubricating oil there is incorporated cobalt naphthenate  $\frac{1}{2}$  per cent and tetramethyl diamino diphenyl methane  $\frac{1}{2}$ -2 per cent and diamino diphenyl methane 0.15 per cent.

As another example: With a similar lubricating oil there is incorporated  $\frac{1}{2}$  per cent of manganese naphthenate and  $\frac{1}{2}$ -2 per cent of tetramethyl diamino diphenyl methane.

As illustrating the properties of such lubricants, the following test-results are noted in summary, in which F is bad or worse than the oil alone, i. e., over 30 mg. of lacquer and over 7 per cent of carbon residue, C is mediocre, i. e., 10-30 mg. of lacquer, and 3.0-7.0 per cent carbon residue, and A is excellent, i. e., less than 10 mg. of lacquer and less than 3.0 per cent of carbon residue.

|                                   | Oil+0.5% Cr naph. | Oil+0.5% Cr naph.+1.5% P <sub>2</sub> S <sub>4</sub> -degas | Oil+0.5% Cr naph.+1.5% tetraphenyl diamino diphenyl methane |
|-----------------------------------|-------------------|-------------------------------------------------------------|-------------------------------------------------------------|
| Carbon residue at—<br>525° F..... | F                 | F                                                           | F                                                           |
| 750° F.....                       | A-                | A-                                                          | C+                                                          |
| Detergency:                       |                   |                                                             |                                                             |
| Carbon suspension.....            | C-                | A                                                           |                                                             |
| Oxidation test.....               | A-                | A                                                           | C+                                                          |
| Oxidation test:                   |                   |                                                             |                                                             |
| Deterioration.....                | A-                | A+                                                          | A                                                           |
| Corrosiveness.....                | A-                | A+                                                          | A                                                           |

The carbon residue is determined by exposing a 2.5 g. sample of the lubricant in a 70 mm. diameter Petri glass dish in an electric furnace for 16 hours at 525° F., followed by 6½ hours at 750° F. The carbon suspension is determined by suspending 5½ per cent by volume of carbon in the lubricant, and a 100 cc. sample of the suspension in a 100 cc. graduate is set in an oven at 200° F., and the number of cc. of clear oil is measured at intervals. The oxidation and lacquer is determined by exposing the lubricant in the presence of metals, iron and copper, at a temperature of 310° F. for 65 hours by blowing air through at the rate of 30 liters per hour.

Other modes of applying the principle of the

invention may be employed, change being made as regards the details described, provided the features stated in any of the following claims, or the equivalent of such, be employed.

5 We therefore particularly point out and distinctly claim as our invention:

1. A lubricant promoting combustion of deposits in the combustion zone of internal combustion engines and producing high stability in the crank-case, which comprises a lubricating oil and up to

10 about three per cent of a salt of an organic acid of low volatility the stated salts of which promote diminution of carbonaceous deposits and a metal having oxidation activity, from the class consisting of vanadium, chromium, molybdenum, manganese, and cobalt, and tetramethyl diamino diphenyl methane and diamino diphenyl methane.

15

2. A lubricant promoting combustion of deposits in the combustion zone of internal combustion engines and producing high stability in the crank-case, which comprises a lubricating oil and up to about three per cent of a salt of an organic acid of low volatility the stated salts of which promote diminution of carbonaceous deposits and a metal having oxidation activity from the class consisting of vanadium, chromium, molybdenum, manganese and cobalt, with a complex organic acid, and a diamino diphenyl methane derivative.

20

3. A process of promoting combustion of deposits in the combustion zone of internal combustion engines and producing high stability in the crank-case, which comprises subjecting oil to internal combustion engine temperature in the presence of up to about three per cent each of a salt of metal having oxidation activity from the class consisting of vanadium, chromium, molybdenum, manganese and cobalt with an organic acid of low volatility the stated salts of which promote diminution of carbonaceous deposits, and

25

40 a nitrogen-containing diphenyl derivative.

4. A lubricant promoting combustion of deposits in the combustion zone of internal combustion engines and producing high stability in the crank-case, which comprises a lubricating oil and up to

45 about three per cent each of a salt of an organic acid of low volatility the stated salts of which promote diminution of carbonaceous deposits with a metal having oxidation activity from the class consisting of vanadium, chromium, molybdenum, manganese and cobalt, and a nitrogen-containing diphenyl methane derivative.

ROBERT E. BURK.  
EVERETT C. HUGHES.